

## 1

3,300,309

MOISTURE-RESISTANT PLANOGRAPHIC PLATES  
AND METHODS OF PRODUCING SAMESimon L. Chu, New York, N.Y., assignor to Polychrome  
Corporation, Yonkers, N.Y.No Drawing. Filed Sept. 6, 1963, Ser. No. 307,025  
18 Claims. (Cl. 96—75)

This invention relates to a novel planographic plate and in particular to a planographic plate comprising a moisture impermeable and light-hardenable coating.

The art of planographic printing depends upon the immiscibility of grease and water, upon the preferential retention of a greasy image-forming substance by the image areas, and a similar retention of an aqueous dampening fluid by the non-image areas. When a greasy image is imprinted upon a suitable surface and the entire surface is then moistened with an aqueous solution, the image areas will repel the water, and the non-image areas will retain the water. Upon subsequent applications of greasy ink, the image portions retain the ink, whereas the moist, non-image areas repel it. The image is then transferred to paper or cloth and so on, etc., via an intermediary so-called offset or blanket cylinder, which is necessary to prevent mirror-image printing.

In the case of negative plates, a plate with a light-sensitive coating is exposed to light through a negative transparency, and the image portion of the plate becomes hard and is made insoluble to desensitizing compositions by the action of the light. The unexposed light-sensitive coating is then removed by a desensitizing solution leaving a water-receptive surface as a non-image area.

The ordinary desensitizing solution used in the art must completely remove the non-sensitized, i.e. non-light hardened, compound. Therefore, this non-light hardened compound must have considerable solubility in desensitizing solutions. It has been a common problem with planographic plates in the art that non-light hardened diazo compounds sufficiently soluble to be completely removed by ordinary desensitizers are also sufficiently permeable to moisture to seriously interfere with the performance of planographic plates by allowing moisture to penetrate the diazo layer, interact with interlayers between the light-sensitive diazo layer and the base plate susceptible to moisture deterioration, and even corrode the metal base plate if the particular planographic plate is metal based. For example, in plates where a  $K_2ZrF_6$ -type interlayer, described in U.S. Patent 2,946,683, lies between a diazo coating and the base, moisture penetrates the diazo coating and reacts with the interlayer in such a way as to cause the bond between the light-hardened material and the remainder of the plate to weaken. This type of action results in "walk-off"; that is, the disappearance of image area during printing. Furthermore, in other types of planographic plates, moisture permeates the diazo coating, reacts chemically with the interlayer, and causes the formation of unwanted image area on the plate, prematurely terminating the usefulness of the plate.

In general, the useful life of presensitized plates coated with diazo compounds is shortened and the performance of such plates is adversely affected by the above-mentioned problems caused by the affinity of these diazo compounds for water. These problems are especially troublesome during periods of high humidity.

It is an object of this invention to provide a moisture-resistant planographic plate having a novel light-hardenable coating which has relatively low affinity for water and which is an intermediate addition product of a diazo with a coupling agent. Another object of the invention is to provide a moisture-resistant coating that is readily removed by ordinary desensitizers known to the art, for example those containing gum arabic, phosphoric acid,

## 2

and a wetting agent like sodium lauryl sulfonate which is sold under the trade name Duponol by E. I. du Pont de Nemours & Company. Another object of the invention is to provide a presensitized plate useful in long press runs because of an improved bonding of the new coating to the remainder of the plate and the improved durability of the coating material when light hardened. It is also an object of this invention to provide a light-sensitive coating for planographic plates that has reduced susceptibility to undesirable chemical reactions during dark storage and thus has an increased shelf life. It is a further object of this invention to provide a novel process by which the novel moisture-resistant coating may be applied to planographic plates.

The novel planographic plates of the present invention comprise a coating which is a product of a reaction between a diazo compound and a coupling agent which reacts with the diazo compound forming, surprisingly, excellent light-sensitive and moisture-resistant coatings. These coatings consist of an intermediate protective compound formed when a light-sensitive diazo is reacted with a coupling agent under such reaction condition that resinification and the resultant formation of a non-light-sensitive compound are avoided. These intermediate compounds, postulated to be addition compounds of the diazo and coupling agent, are sufficiently resistant to moisture permeation to eliminate the aforementioned problems of specking, toning, and walk-off in normal, and even severe heat and humidity.

Diazo compounds of the type commonly used in the planographic plate industry are resinified when reacted with a coupling agent in excessively basic medium. Such a reaction is of no value as a method of forming a protective coating for a planographic plate inasmuch as it destroys the light-sensitive potential of the diazo compound. However, applicant has discovered that coupling agents reacted in relatively acid media form a novel moisture-resistant intermediate azo addition product which also has the light-sensitive character of the original diazo compound.

Applicant has further discovered that such products are resistant to "dark reactions," i.e. reactions occurring without exposure to light, have increased press life, and generally provide most excellent coatings for planographic printing plates.

The number of coupling agents useful for the purposes of this invention is large. They are best described by a recitation of their main characteristic, i.e. an ability to react with the chosen diazo under reaction conditions that will not cause resinification and resultant loss of the reaction products' light-sensitive characteristics. Those coupling agents reacting with the diazo in an acid medium, i.e. at a pH of about 7.5 or below, are found to be especially advantageous for the practice of the instant invention.

Among the coupling agents that are suitable for use in the reaction of the present invention are hydroxy benzophenones, diphenolic acids such as 4,4-bis(4-hydroxyphenyl)pentanoic acid, resorcinol, diresorcinol, 1-naphthol-3-sulfonamide, 2-naphthol-3,6-disulfonic acid disodium salt and N-alkyl-5-sulfonanthranilic acids such as the methyl and ethyl compounds. These materials may have as substituents groups such as aldehyde, carboxyl or sulfonic groups. Group tending to impart water-solubility are favored whereas those tending to impart water-insolubility are less desirable unless their effect is counterbalanced. In fact, very little water solubility, perhaps 0.05 percent, is required of the coupling agent at normal reaction temperatures. Among the hydroxy benzophenones suitable for the present invention are 2,4-dihydroxy-benzophenone, 2-hydroxy-4-methoxy-benzophenone, 2,2'-dihydroxy-4,4'-dimethoxy-benzophenone, 2,2',

4,4'-tetrahydroxy-benzophenone, sodium 2,2'-dihydroxy-4,4'-dimethoxy-5-sulfobenzophenone, 2-hydroxy-4-methoxy-benzophenone-5-sulfonic acid, the trihydrate of the last-named acid, and mixtures of such compounds.

The 2,2'-4,4'-tetrahydroxy-benzophenone is preferred among these compounds.

The diazo compounds conveniently used as reactants with the above-identified coupling agents are of the type useful on planographic printing plates generally and which are capable of reacting with the coupling agent at a pH sufficiently low to avoid forming a resinified reaction product with the coupling agent, i.e. a product which has insufficient sensitivity to light to remain useful as a planographic plate coating. Among such compounds are the condensation products of para-diazo-diphenyl-amine and formaldehyde, for example, the condensation product of para-diazo-diphenyl-amine sulfate and formaldehyde zinc chloride, and the diazo compound sold by Fairmont Chemical Co., Inc. under the trade designation Diazo Resin No. 4 as well as other diazos which are well known to those skilled in the art.

In one embodiment of the instant invention, the planographic plate, initially having a top coating of the conventional diazo compounds known to the art, is coated with a solution of the coupling agent. This solution, in which the diazo is somewhat soluble, will preferably contain from 0.01 to 0.5% of the coupling agent and, preferably, small quantities of additives such as a wetting agent or a polyhydroxy acid. This solution is coated on the diazo layer and reacts therewith forming the intermediate azo addition compound. Depending on circumstances such as concentration, temperature and the particular solvent employed, the reaction will be very nearly instantaneous or it may take up to several minutes or more. The product of the foregoing reaction is the light-hardenable reaction product which is exceedingly well bonded to the plate and thus has a longer press life than diazo coated planographic plates even before storage deterioration.

In another embodiment of the present invention, the diazo and coupling compounds are reacted in a solvent. The solution containing the light-sensitive intermediate azo product so formed is coated on the interlayer of the planographic plates. Upon the evaporation of the solvent, the moisture-resistant diazo polymer coating remains on the plate.

In this latter embodiment, the reaction normally has a greater time in which to proceed. Thus the most impermeable and resistant coatings may be achieved.

Solvents in which the reaction may be advantageously

num and copper are among the more suitable metals. Furthermore, plastic and paper base members are also suitable for use in constructing planographic plates of the present invention.

5 Various metal-protective coatings may be used as interlayers between the light-sensitive coating and metal base member. Among such interlayers are aluminum oxide (for example, as found in anodized aluminum plates), the reaction products of an aqueous solution of soluble silicate with the metal base, and reaction products of aqueous solutions of zirconium hexahalides, like potassium zirconium hexachloride, with the metal base. All of these illustrative interlayers are known to the art.

In order to point out more fully the nature of the present invention, the following specific examples are given as various embodiments of the present process and products produced thereby.

#### Example 1

20 An aluminum offset plate 10 inches by 15 inches and .005-inch thick was coated consecutively with a  $K_2ZrF_6$  coating and a light-sensitive diazo compound according to U.S. Patent 2,946,683.

25 A water solution was prepared containing 0.1% saponin and 0.5% 2,2',4,4'-tetrahydroxy-benzophenone. This solution was coated over the planographic plate. After a contact time between solution and plate of one to two seconds, the excess solution was wiped off from the plate and the plate was dried, leaving the plate coated with the reaction product of the diazo and 2,2',4,4'-tetrahydroxy-benzophenone.

30 The plate prepared at about 20-50° C. as indicated above was exposed to a high humidity environment in a chamber with a number of other pre-sensitized lithographic plates having conventional diazo coatings and otherwise characterized as follows:

Plate A is a commercially-available plate having a diazo coating.

35 Plate B is a plate comprising a silicate layer interposed between the aluminum base plate and a diazo layer, the manufacture of which is described in U.S. Patent 2,922,715.

40 Plate C is a plate comprising a  $K_2ZrF_6$  interlayer between a diazo coating and an aluminum base and differs from the plate prepared in accordance with this example only in the light-sensitive coating used.

The plates subjected to the test were exposed at 90° F. and 90% relative humidity.

The results of the test are shown in the following table:

#### CONDITION OF PLATE

|              | Plate of Ex. 1    | A                                    | B                                              | C                                   |
|--------------|-------------------|--------------------------------------|------------------------------------------------|-------------------------------------|
| 3 days.....  | Satisfactory..... | Satisfactory.....                    | Satisfactory.....                              | Unsatisfactory; excessive walk off. |
| 7 days.....  | do.....           | Specking, unsatisfactory.<br>do..... | Specking, unsatisfactory.<br>do.....           |                                     |
| 14 days..... | do.....           |                                      | Specking and toning, unsatisfactory.           |                                     |
| 28 days..... | do.....           |                                      | Corrosion and toning on plate, unsatisfactory. |                                     |
| 45 days..... | do.....           |                                      | Corrosion and toning on plate, unsatisfactory. |                                     |

carried out include, for example, water, alcohols such as lower alkyl alcohols, acetates such as ethyl acetate, and lower alkyl ketones. The common commercial grades of these solvents are used advantageously and, in deed, water contained therein is useful in promoting the desired reaction. Mixtures of the aforementioned solvents may also be used. When such solvents as acetates and ketones are used, it is preferable to include in the solvent mixture quantities of water, preferably about 20 to 80% of the solvent. Methanol and water are two preferred solvents for use in the present invention.

As is known in the art, various metals may be used for base members for planographic plates. Zinc, alumi-

65 Upon treating Plates A, B and C with 2,2',4,4'-tetrahydroxy-benzophenone as described above, they too remained in satisfactory condition for 45 days when subjected to the indicated humidity and heat environment.

Anodized plates, mechanically grained plates, and even paper plates were also improved in moisture resistance and overall performance when coated with the intermediate azo reaction product of the present invention.

#### Example 2

75 An aluminum offset plate 10 inches by 15 inches and .005-inch thick was coated, consecutively with a  $K_2ZrF_6$

coating and a light-sensitive diazo compound according to U.S. Patent 2,946,683.

A water solution was prepared containing 0.1% saponin and 0.25 diresorcinol. This solution was coated over the planographic plate. After a contact time between solution and plate of one to two seconds, the excess solution was wiped from the plate and the plate was dried.

An azo addition product resin coated the surface which was light-hardenable and impermeable to moisture as indicated by its remaining in satisfactory condition even when subjected to 90% relative humidity and 90° F. for 45 days and testing as follows:

The plate was removed from the high humidity environment, exposed to light through a negative transparency, desensitized with a conventional desensitizing agent, coated with a protective lacquer, and mounted upon a press. The run was successful, being discontinued after 8000 prints were run off. The last copies were still excellent, indicating the fine performance of the plate.

#### Example 3

An aluminum offset plate 10 inches by 15 inches and .005-inch thick was coated, consecutively with a  $K_2ZrF_6$  coating and a light-sensitive diazo compound according to U.S. Patent 2,946,683.

An isopropanol solution was prepared containing 0.1% saponin and 0.05% sodium 2,2'-dihydroxy-4,4'-dimethoxy-5-sulfobenzophenone. This solution was coated over the planographic plate. After a contact time between solution and plate of one to two seconds, the excess solution was wiped from the plate and the plate was dried.

An azo addition product coated the surface which was light-hardenable and impermeable to moisture as indicated by its remaining in satisfactory condition even when subjected to 90% relative humidity and 90° F. for 45 days and its performing well in the test described in Example 2.

#### Example 4

An aluminum offset plate 10 inches by 15 inches and .005-inch thick was coated, consecutively with a  $K_2ZrF_6$  coating and a light-sensitive diazo compound according to U.S. Patent 2,946,683.

A 50% butyl acetate and 50% water solution was prepared containing 0.1% saponin and 0.25% 2,2',4,4'-tetrahydroxy-benzophenone. This solution was coated over the planographic plate. After a contact time between solution and plate of one to two seconds, the excess solution was wiped from the plate and the plate was dried.

An azo addition product coated the surface which was light-hardenable and impermeable to moisture as indicated by its remaining in satisfactory condition even when subjected to 90% relative humidity and 90° F. for 45 days and its performing well in the test described in Example 2.

#### Example 5

An aluminum offset plate 10 inches by 15 inches and .005-inch thick was coated, consecutively with a  $K_2ZrF_6$  coating and a light-sensitive diazo compound according to U.S. Patent 2,946,683.

A 50% acetone and 50% water solution was prepared containing 0.1% saponin and 0.40% N-ethyl-5-sulfoanthranilic acid. This solution was coated over the planographic plate. After a contact time between solution and plate of one to two seconds, the excess solution was wiped from the plate and the plate was dried.

An azo addition product coated the surface which was light-hardenable and impermeable to moisture as indicated by its remaining in satisfactory condition even when subjected to 90% relative humidity and 90° F. for 45 days and its performing well in the test described in Example 2.

#### Example 6

An aluminum offset plate 10 inches by 15 inches and .005-inch thick was coated, consecutively with a  $K_2ZrF_6$

coating and a light-sensitive diazo compound according to U.S. Patent 2,946,683.

A 90% water and 10% ethanol solution was prepared containing 0.1% saponin and 0.15% 4,4-bis(4-hydroxy-phenyl) pentanoic acid. This solution was coated over the planographic plate. After a contact time between solution and plate of one to two seconds, the excess solution was wiped from the plate and the plate was dried.

An azo addition product coated the surface which was light-hardenable and impermeable to moisture as indicated by its remaining in satisfactory condition even when subjected to 90% relative humidity and 90° F. for 45 days and its performing well in the test described in Example 2.

#### Example 7

An aluminum offset plate 10 inches by 15 inches and .005-inch thick was coated, consecutively with a  $K_2ZrF_6$  coating and a light-sensitive diazo compound according to U.S. Patent 2,946,683.

A methanol solution was prepared containing 0.1% saponin and 0.30% 1-naphthol-3-sulfonamide. This solution was coated over the planographic plate. After a contact time between solution and plate of one to two seconds, the excess solution was wiped from the plate and the plate was dried.

An azo addition product coated the surface which was light-hardenable and impermeable to moisture as indicated by its remaining in satisfactory condition even when subjected to 90% relative humidity and 90° F. for 45 days and its performing well in the test described in Example 2.

#### Example 8

An aluminum offset plate 10 inches by 15 inches and .005-inch thick was coated with a  $K_2ZrF_6$  coating according to U.S. Patent 2,946,683.

Five parts by volume water solution containing 2% of the diazo compound were mixed into four parts of isopropyl alcohol containing 5 grams of 2,2',4,4'-tetrahydroxy benzophenone. One part water was added to the mix, and the plate was coated therewith.

Upon wiping off the excess solvent and drying the plate, an azo addition compound coated the surface which was light-hardenable and impermeable to moisture as indicated by its remaining in satisfactory condition even when subjected to 90% relative humidity and 90° F. for 45 days and its performing well in the test described in Example 2.

It is of course to be understood that the foregoing examples are intended to be illustrative and that various changes can be made in the ingredients, proportions, and conditions set forth therein without departing from the spirit of the invention as defined in the appended claims.

I claim:

1. A moisture-resistant planographic plate which comprises a base member having coated thereon a light-sensitive, moisture-resistant compound that is the reaction product of a light-sensitive diazonium compound and a phenolic hydroxyl-containing aromatic coupling agent formed in a medium having a pH of less than about 7.5 substantially to prevent resinification.

2. A moisture-resistant planographic plate which comprises a base member having coated thereon a light-sensitive moisture-resistant compound that is the reaction product of (a) a light-sensitive diazonium compound obtained by the reaction of a diazo compound and a reactive carbonyl-containing compound and (b) a phenolic coupling agent formed in a medium having a pH of less than about 7.5 substantially to prevent resinification.

3. A moisture-resistant planographic plate which comprises a base member having coated thereon a light-sensitive moisture-resistant compound that is the reaction product of (a) a light-sensitive diazonium compound obtained by the reaction of a diazo-diphenylamine and formaldehyde and (b) a phenolic compound, said reac-

tion product being formed at a pH of less than about 7.5 substantially to prevent resinification.

4. A moisture-resistant planographic plate which comprises a base member having coated thereon a light-sensitive moisture-resistant compound that is the reaction product of (a) a light-sensitive diazonium compound obtained by the reaction of a diazo-diphenylamine and formaldehyde and (b) a phenolic compound selected from the group consisting of hydroxybenzophenones, diphenolic alkanoic acids, dihydroxy-benzenes, tetrahydroxy-biphenyls, naphthol sulfonamides, naphthol sulfonic acids, naphthol sulfonic acid salts and sulfantranilic acids, said reaction product being formed at a pH of less than about 7.5 substantially to prevent resinification.

5. A moisture-resistant planographic plate which comprises a base member having coated thereon a light-sensitive moisture-resistant compound that is the reaction product of (a) a light-sensitive diazonium compound obtained by the condensation of para-diazo-diphenylamine sulfate with formaldehyde zinc chloride and (b) a coupling agent selected from the group consisting of 4,4-bis(4-hydroxyphenyl)-pentanoic acid, resorcinol, diresorcinol, 1 - naphthol-3-sulfon-amide, 2-naphthol-3,6-disulfonic acid disodium salt, N-lower alkyl-5-sulfoanthranilic acid, 2,4-dihydroxy-benzophenone, 2-hydroxy-4-methoxy-benzophenone, 2,2' - dihydroxy - 4,4'-dimethoxy-benzophenone, 2,2',4,4'-tetrahydroxy-benzophenone, sodium 2,2' - dihydroxy - 4,4'-dimethoxy-5-sulfonylbenzophenone, 2-hydroxy - 4 - methoxy-benzophenone-5-sulfonic acid and 2-hydroxy-4-methoxy-benzophenone-5-sulfonic acid trihydrate, said reaction product being formed at a pH of less than about 7.5 substantially to prevent resinification.

6. A method for the preparation of a storage-stable, light-sensitive, moisture-resistant planographic plate which comprises coating a base for said planographic plate with a light-sensitive, moisture-resistant compound that is the reaction of a light-sensitive diazonium compound and a phenolic hydroxyl-containing aromatic coupling agent formed in a medium having a pH of less than about 7.5 substantially to prevent resinification.

7. A method for the preparation of a storage-stable, light-sensitive, moisture-resistant planographic plate which comprises coating a base for said planographic plate with a light-sensitive moisture-resistant compound that is the reaction product of (a) a light-sensitive diazonium compound obtained by the reaction of a diazo compound and a reactive carbonyl-containing compound and (b) a phenolic coupling agent formed in a medium having a pH of less than about 7.5 substantially to prevent resinification.

8. A method for the preparation of a storage-stable, light-sensitive, moisture-resistant planographic plate which comprises coating a base for said planographic plate with a light-sensitive moisture-resistant compound that is the reaction product of (a) a light-sensitive diazonium compound obtained by the reaction of a diazo-diphenylamine and formaldehyde and (b) a phenolic compound, said reaction product being formed at a pH of less than about 7.5 substantially to prevent resinification.

9. A method for the preparation of a storage-stable, light-sensitive, moisture-resistant planographic plate which comprises coating a base for said planographic plate with a light-sensitive moisture-resistant compound that is the reaction product of (a) a light-sensitive diazonium compound obtained by the reaction of a diazo-diphenylamine and formaldehyde and (b) a phenolic compound selected from the group consisting of hydroxybenzophenones, diphenolic alkanoic acids, dihydroxy-benzenes, tetrahydroxy-biphenyls, naphthol sulfonamides, naphthol sulfonic acids, naphthol sulfonic acid salts and sulfantranilic acids, said reaction product being formed at a pH of less than about 7.5 substantially to prevent resinification.

10. A method for the preparation of a storage-stable,

light-sensitive, moisture-resistant planographic plate which comprises coating a base for said planographic plate with a light-sensitive moisture-resistant compound that is the reaction product of (a) a light-sensitive diazonium compound obtained by the condensation of para-diazo-diphenylamine sulfate with formaldehyde zinc chloride and (b) a coupling agent selected from the group consisting of 4,4-bis(4-hydroxyphenyl)-pentanoic acid, resorcinol, diresorcinol, 1 - naphthol - 3 - sulfon - amide, 2-naphthol - 3,6 - disulfonic acid disodium salt, N - lower alkyl - 5 - sulfoanthranilic acid, 2,4 - dihydroxy - benzophenone, 2 - hydroxy - 4 - methoxy - benzophenone, 2,2' - dihydroxy - 4,4' - dimethoxy - benzophenone, 2,2',4,4'-tetrahydroxy - benzophenone, sodium 2,2' - dihydroxy - 4,4'-dimethoxy-5-sulfonylbenzophenone, 2-hydroxy - 4 - methoxy-benzophenone-5-sulfonic acid and 2-hydroxy-4-methoxy-benzophenone-5-sulfonic acid trihydrate, said reaction product being formed at a pH of less than about 7.5 substantially to prevent resinification.

11. A method for the preparation of a storage-stable, light-sensitive, moisture-resistant planographic plate which comprises coating a base for said planographic plate, with a light-sensitive diazonium compound, applying a phenolic hydroxyl-containing aromatic coupling agent to said diazonium-coated base at a pH of below about 7.5 to form a substantially unresinified light-sensitive moisture-resistant reaction product, and removing unreacted residues from said plate.

12. A method for the preparation of a storage-stable, light-sensitive, moisture-resistant planographic plate which comprises coating a base for said planographic plate with a light-sensitive diazonium compound obtained by the reaction of a diazo compound and a reactive carbonyl-containing compound, applying a phenolic coupling agent to said diazonium-coated base at a pH of below about 7.5 to form a substantially unresinified light-sensitive moisture-resistant reaction product, and removing unreacted residues from said plate.

13. A method for the preparation of a storage-stable, light-sensitive, moisture-resistant planographic plate which comprises coating a base for said planographic plate with a light-sensitive moisture-resistant compound that is the reaction product of a light-sensitive diazonium compound obtained by the reaction of a diazo-diphenylamine and formaldehyde, applying a phenolic coupling agent to said diazonium-coated base at a pH of below about 7.5 to form a substantially unresinified light-sensitive moisture-resistant reaction product, and removing unreacted residues from said plate.

14. A method for the preparation of a storage-stable, light-sensitive, moisture-resistant planographic plate which comprises coating a base for said planographic plate with a light-sensitive diazonium compound obtained by the reaction of diazo-diphenylamine and formaldehyde, applying a phenolic coupling agent selected from the group consisting of hydroxybenzophenones, diphenolic alkanoic acids, dihydroxy-benzenes, tetrahydroxy-biphenyls, naphthol sulfonamides, naphthol sulfonic acids, naphthol sulfonic acid salts and sulfantranilic acids to said diazonium-coated base at a pH of below about 7.5 to form a substantially unresinified light-sensitive moisture-resistant reaction product, and removing unreacted residues from said plate.

15. A method for the preparation of a storage-stable, light-sensitive, moisture-resistant planographic plate which comprises coating a base for said planographic plate with a light-sensitive diazonium compound obtained by the condensation of para-diazo-diphenylamine sulfate with formaldehyde zinc chloride, applying a phenolic coupling agent selected from the group consisting of 4,4-bis(4-hydroxyphenyl)-pentanoic acid, resorcinol, diresorcinol, 1 - naphthol - 3 - sulfon - amide, 2 - naphthol - 3,6 - disulfonic acid disodium salt, N - lower alkyl - 5 - sulfoanthranilic acid, 2,4 - dihydroxy - benzophenone, 2 - hydroxy - 4 - methoxy - benzophenone, 2,2' - dihydroxy - 4,4' - dimethoxy - benzophenone, 2,2',4,4'-tetrahydroxy - benzophenone, sodium 2,2' - dihydroxy - 4,4'-dimethoxy-5-sulfonylbenzophenone, 2-hydroxy - 4 - methoxy-benzophenone-5-sulfonic acid and 2-hydroxy-4-methoxy-benzophenone-5-sulfonic acid trihydrate, said reaction product being formed at a pH of less than about 7.5 substantially to prevent resinification.

hydroxy - 4 - methoxy - benzophenone, 2,2' - dihydroxy - 4,4' - dimethoxy - benzophenone, sodium - 2,2' - dihydroxy - 4,4' - dimethoxy - 5 - sulfobenzophenone, 2 - hydroxy 4 - methoxybenzophenone - 5 - sulphonic acid and 2 - hydroxy - 4 - methoxy - benzophenone - 5 - sulfonic acid trihydrates to said diazonium-coated base at a pH of below about 7.5 to form a substantial unresinified light-sensitive moisture-resistant reaction product, and removing unreacted residues from said plate.

16. A moisture-resistant planographic plate which comprises a base member having coated thereon a light-sensitive, moisture-resistant compound that is the reaction product of a light-sensitive diphenylamine diazonium compound and a phenolic hydroxyl-containing aromatic coupling agent formed in a medium having a pH of less than about 7.5 substantially to prevent resinification.

17. A method for the preparation of a storage-stable, light-sensitive, moisture-resistant planographic plate which comprises coating a base for said planographic plate with a light-sensitive, moisture-resistant compound that is the reaction product of a light-sensitive diphenylamine diazonium compound and a phenolic hydroxyl-containing aromatic coupling agent formed in a medium

having a pH of less than about 7.5 substantially to prevent resinification.

18. A method for the preparation of a storage-stable, light-sensitive, moisture-resistant planographic plate which comprises coating a base for said planographic plate with a light-sensitive diphenylamine diazonium compound, applying a phenolic hydroxyl-containing aromatic coupling agent to said diazonium-coated base at a pH of less than about 7.5 to form a substantially unresinified light-sensitive moisture-resistant reaction product, and removing unreacted residue from said plate.

#### References Cited by the Examiner

##### UNITED STATES PATENTS

|    |           |         |                   |       |       |
|----|-----------|---------|-------------------|-------|-------|
| 15 | 2,702,242 | 2/1955  | Neugebauer et al. | ---   | 96-33 |
|    | 2,946,683 | 7/1960  | Mellan et al.     | ----- | 96-33 |
|    | 3,169,864 | 2/1965  | Holmen            | ----- | 96-75 |
|    | 3,186,845 | 6/1965  | Sus et al.        | ----- | 96-75 |
| 20 | 3,210,184 | 10/1965 | Uhlig             |       |       |

J. TRAVIS BROWN, *Acting Primary Examiner.*

ALEXANDER D. RICCI, *Examiner.*